

No. 660,932.

Patented Oct. 30, 1900.

W. H. A. SIEVERTS.  
MANTLE FOR INCANDESCENT LAMPS.

(Application filed May 20, 1899.)

(No Model.)



Witnesses:

*W.C. Keeley*  
*Anthony J. Sargeant*

Inventor  
Wilhelm H. A. Sieverts  
By  
*James L. Norris*  
atty

# UNITED STATES PATENT OFFICE

WILHELM HEINRICH AUG. SIEVERTS, OF HAMBURG, GERMANY.

## MANTLE FOR INCANDESCENT LAMPS.

SPECIFICATION forming part of Letters Patent No. 660,932, dated October 30, 1900.

Application filed May 20, 1899. Serial No. 717,592. (No model.)

*To all whom it may concern:*

Be it known that I, WILHELM HEINRICH AUGUST SIEVERTS, teacher, a subject of the Emperor of Germany, residing at Hamburg-5 Uhlenhorst, in the Empire of Germany, have invented an Improved Mantle for Incandescent Lamps, of which the following is a specification.

This invention relates to mantles for incandescent lamps; and it has for its object to provide a new and improved mantle which is more elastic than the ordinary mantle, is strengthened in a novel manner at the part which usually bears or rubs against the burner, and at other parts, if desired, the meshes are enabled to slide one in the other prior to burning to obtain elasticity, the mantle possesses a high coefficient expansion and rapidly expands when lighted, and the illuminating power of the mantle is materially increased. This object is accomplished in the manner and by the means hereinafter described and claimed, reference being made to the accompanying drawings, in which—

25 Figure 1 shows a mantle strengthened by thicker meshes saturated with a thicker coating at the portion between *a* and *b* where it may come into contact with the burner. Fig. 2 shows a portion of the weaving of the mantle provided with thick mesh extending from *c* to *d*. Fig. 3 shows a mantle drawn inwardly by the action of the flame and which touches the edge of the burner at *a a*. Fig. 4 shows a mantle constructed in accordance 30 with this invention, as shown separately in Fig. 1, mounted upon a Bunsen burner. Fig. 5 shows a mantle constructed in accordance with this invention which is strengthened by thicker meshes and a thicker coating by saturation at its upper end between *e* and *f*, at its middle portion between *g* and *h*, and at the portion surrounding the burner between *i* and *k*.

The object of the invention is to produce a 45 mantle for incandescence which (*a*) forms an elastic instead of a rigid body as heretofore and (*b*) is strengthened in the vicinity of the top edge of the burner, so as to enable the mantle to resist the sucking action of the 50 flame, together with the outer pressure of the air, and (*c*) is formed with a convex portion

at the top edge of the burner, so as to prevent it coming into contact therewith.

Careful study in the manufacture of incandescent mantles has led me to discover 55 that, first, the finished mantle has a strong high coefficient expansion, and thus when being lighted it rapidly expands for several millimeters, while shrinking again on being extinguished, and, second, the incandescent 60 mantle loses much of its rigidity by a repeated steeping of the fabric before burning it, inasmuch as the meshes are thereby enabled to slide the one in the other to a certain extent. The phenomenon mentioned 65 under No. 1 is the reason that the slightly-built and rigid weaving forming the mantle is drawn in by the sucking action of the flame and by the pressure of the air-current which passes through the meshes into the flame, and 70 so comes into contact with the top edge of the burner, as indicated at *a a* in Fig. 3 of the drawings, and is thus damaged or breaks at that point. The peculiar movement of the meshes mentioned under No. 2 was entirely 75 unknown heretofore and may be explained as being a consequence of the immediate burning of the mantle after a second steeping of the zone which it is desired to strengthen. The reason for the phenomenon is deduced from 80 the well-known fact that when a small piece of thorium nitrate is placed in a flame it becomes puffed up to a large extent, owing to the escape of the nitric acid therefrom. By steeping the fabric in strong solution and 85 then burning the woven fabric before it has time to dry completely a portion of the dissolved thorium nitrate separates before it can be fixed by the fabric and appears thereon in the form of minute white pearls. The 90 nitric acid which escapes therefrom causes these pearls to puff up, and thereby prevents the sintering together of the thorium sucked up by the threads and keeps it perfectly free (not sintered together) at the points of intersection of the burned-out skeleton. The 95 knowledge thus gained from these facts has led to the discovery of an incandescent mantle which by an extra amount of steeping in strong solution is rendered elastic, and thereby more able to withstand vibrations 100 and which is further constructed with an out-

wardly-curved zone of thicker meshes at the part surrounding the top edge of the burner in order to prevent it being damaged by coming into contact with the top of the said burners. The strong solution is prevented from spreading beyond the zone by capillary action either by quickly drying the part or by burning it immediately. A mantle thus treated when placed over the gas-flame bulges out by itself by reason of the remaining or non-treated portion of the mantle shrinking to a greater extent than that of the zone which has been dipped in the strong solution.

Any known means may be utilized for producing stronger threads at the desired part of a mantle. Thus, for instance, the spun threads may be more twisted at some places than at others. Such threads enable a cylindrical or hose fabric to be manufactured having at certain parts thick meshes, such as shown at *d*, Fig. 2. This is then cut to the desired length for the mantles, which are thereupon treated in the well-known manner.

Another disadvantage in connection with the existing mantles is that they contract at the top after short service, and this contraction detracts greatly from the illuminating power of the mantle, owing to the surface being reduced thereby and the mantle being no longer at the periphery of the flame. This is also due to the sucking of the flame, and it

may be avoided by forming a strengthening zone *g h*, Fig. 5, parallel to the one near the top of the burner by meshes of greater thickness and a thicker coating by saturation, as 35 before described. It is also advantageous to strengthen the top portion or top edge of the mantle, as shown at *e f*, Fig. 5.

Mantles thus constructed keep their form, and thus retain their illuminating power for 40 a longer period, while the increased deposition of materials at the portions most affected by the flame gives greater brilliancy in the light.

What I claim is—

As an improved article of manufacture, an elastic mantle of a single layer of woven material having a zone formed of threads of greater thickness than the threads composing the body of the mantle, said thickened zone 50 being more heavily coated with incandescent material than, and with the same incandescent material as, the other portions of the mantle, substantially as described and for the purpose specified.

In testimony whereof I have hereunto set my hand, in presence of two subscribing witnesses, this 9th day of May, 1899.

WILHELM HEINRICH AUG. SIEVERTS.

Witnesses:

WILHELM FRENZ,  
JULIUS HAND.

45

55